

## UNITED STATES PATENT OFFICE.

FELIX KIRSCHNER, OF VIENNA, AUSTRIA.

## PROCESS FOR THE PRODUCTION OF GALVANIC METAL COATINGS.

No Drawing. Application filed October 12, 1923, Serial No. 668,162, and in Austria June 19, 1923.

The present invention relates to a process for the production of galvanic coatings, which is remarkable for the high quality of the goods produced and the economy with which the process can be carried out. It has been found that galvanic coatings which are deposited upon a metallic intermediate coating alloyed to the basic metal of the article, possess surprising qualities as regards appearance, adherence, density, hardness, polish and resistance to chemical and mechanical influences. With the new process, new alloy coated goods (galvano-alloyed goods) can be produced and numerous forms of plating which hitherto could only be obtained by means of difficult and costly processes (nickel plating, silver plating and the like) can be effected in a simple manner and of a technically high quality.

One application of the new process is described below in connection with the production of galvanic nickel plating.

The goods to be nickel plated are for example first galvanically provided with a metal coating of pure tin or an alloy or alloys containing tin. The intermediate coating of tin or tin alloy thus applied is then fused on by the application of heat and other known means, so that the intermediate layer after hardening has a smooth bright and glossy surface. During the fusing of the intermediate layer the deposited metal (tin or tin alloy) becomes alloyed with the basic metal (e. g. iron or copper) of the goods. This intermediate product, having for example a body of iron or copper has a surface of pure deposited metal (tin) with a smooth bright and glossy surface, whilst where the deposited metal adjoins the basic metal of the article there is formed an alloy of the basic metal with the tin or tin alloy that has been deposited.

It is particularly advantageous to alloy the galvanically applied intermediate layer (for example tin) with the basic metal and to provide it with a bright and glossy surface in the following manner. The galvanically applied intermediate layer upon the goods is fused with the assistance of known flux agents (for example of dilute acids, ammonium chloride with or without the addition of metal salts) and is cooled in a water bath in a manner suited to the specific manner of cooling of the fused metal.

If nickel is galvanically deposited upon the intermediate product thus obtained, it is found that the nickel coating, without the usual elaborate preparation that is necessary for nickel plating (for example, grinding, polishing, brushing, burnishing and coppering), is immediately obtained with surprising closeness, adherence and brightness.

It is advantageous to carry out the galvanic nickel plating immediately after the water cooling of the intermediate layer, that is to say whilst the goods are still wet. Particularly good and bright effects can be obtained if the goods, after the hardening of the intermediate fused layer has been effected by cooling and before the galvanic covering coating is applied, are submitted to treatment with weak acids, e. g. weak sulphuric acid.

The above described example of the process for nickel plating can be varied in many different ways. Instead of using the galvanically produced and subsequently fused intermediate layer which is alloyed with the basic metal, any other process such as a dipping or boiling process known for obtaining the metallic intermediate layer can be employed, wherein the alloying between the basic metal and the intermediate layer is effected by thermic treatment.

The following is a further example of how the invention may be applied for galvanic silver plating, coating with brass or the like.

In this process a metallic intermediate layer of pure tin or tin alloy is applied to the basic metal by any known dipping process, galvanic process or boiling process. This intermediate layer is given a bright surface by being subjected to heat, either from a flame, or from electric resistances or from a source of radiant heat, and it is alloyed with the basic material. Upon this alloyed intermediate layer metallic outer coatings, two or more in number, can with great advantage be successfully applied.

The alloying of the intermediate layer with the basic metal and the production of a smooth and glossy surface can with particular advantage be obtained by fusing the galvanically applied coating of the intermediate layer with the assistance of fluxes such for example as mixtures of weak acids and ammonium chloride with or without the

addition of metal salts, the fusing being cooled with water according to the specific manner of hardening of the fused metal. In silver plating, nickel is first deposited galvanically upon the glossy surface of the intermediate layer alloyed with the basic metal and silver is afterwards deposited.

It has been found that with the above described process silver goods can be produced with only a very thin coating of silver and that they retain their good appearance for a very long time; this appears to be due to the provision of the hard glossy nickel under coating. But even where a heavy coating of silver is applied to a basic metal that is not white, for example, brass or pinchbeck, the present process is of considerable value.

For applying a coating of brass or pinchbeck, nickel is first of all galvanically applied to the intermediate layer of metal alloyed with the basic metal and thereupon

brass or pinchbeck is deposited by means of any known process.

What I claim is:

1. The herein described method of producing a highly lustrous metallic coating upon a metal base, which consists in electrolytically coating the ground metal with a layer of low-melting-point metal, fusing the layer to the ground metal and thereupon cooling it in a water solution to transform it into a layer having a smooth highly lustrous surface, and immediately electrolytically depositing nickel thereupon. 30 35

2. The herein described method as set forth in claim 1, in which the low-melting-point metal consists of tin.

3. In the herein described method as set forth in claim 1, the additional step of electrolytically depositing a further metal upon the nickel coating. 40

In testimony whereof I affix my signature.

FELIX KIRSCHNER.